# EUROPEAN PATENT APPLICATION

(11) **EP 0 808 681 A1**
(43) Date of publication of application: **26.11.1997**
(21) Application number: 96935351.5
(22) Date of filing: 17.10.1996
(51) Int. Cl.: B22F 1/00, B22F 9/08, C22C 33/02, C22C 38/00

(54) **IRON POWDER FOR POWDER METALLURGY, PROCESS FOR PRODUCING THE SAME, AND IRON-BASE POWDER MIXTURE FOR POWDER METALLURGY**

(30) Priority: 18.10.1995 JP 270275/95
(71) Applicant: KAWASAKI STEEL CORPORATION, Chuo-ku, Kobe-shi, Hyogo 651 (JP); MITSUBISHI MATERIALS CORPORATION, Chiyoda-ku, Tokyo 100 (JP)
(72) Inventor: UENOSONO, Satoshi, Tech. Res. Lab., Chiba-shi, Chiba-ken 260 (JP); OGURA, Kuniaki, Tech. Res. Lab., Chiba-shi, Chiba-ken 260 (JP); YANG, Ji-bin, Niigata Plant, Niigata-shi, Niigata-ken 950 (JP)
(74) Representative: Lindgren, Anders
(86) International application number: JP9603007
(87) International publication number: WO9714523

(57) **Abstract**

An object of the present invention is to provide iron powders for powder metallurgy and iron base mixed powders capable of producing sintered bodies excellent in machinability and abrasion resistance. Such an object is solved in accordance with the following means.

There is provided an iron powder comprising 0.03-0.3 wt% of B, not larger than 0.07 wt% of Cr, less than 0.3 wt% of Mn, and a balance being Fe and inevitable impurities, and an intensity ratio of B to Fe as to an emission spectrum obtained through a measurement on a surface of the iron powder according to Auger electron spectroscopy is not less than 0.05. The use of this iron powder causes an amount of residual graphite in sintered bodies to increase thereby improving machinability and abrasion resistance of the sintered bodies. Further, there is provided an iron powder which comprises S, Se, Te and/or Mo in addition to the above-mentioned compositions. Furthermore, there is developed a so-called iron base mixed powder in which MoO₃ powder and/or WO₃ powder are mixed with said iron powders. These iron powders are produced in such a manner that in addition to the above-mentioned compositions, particularly, an amount of oxygen in a molten steel is controlled to be not more than 100 ppm, and the molten steel is water-atomized.

## Description

### Technical Field

The present invention relates to iron powders for powder metallurgy, a method of producing the iron powders, and iron base mixed powders for powder metallurgy, and more particular to powders which exhibit excellent machinability and abrasion resistance when the powders are sintered.

### Background Art

In general, the powder metallurgy is a technology as to the production of massive materials and shaped objects by pressing, binding, and sintering powdered metal. For example, in a case where iron powder is adopted as the powdered metal, copper powder and graphite powder are mixed with the iron powder and the mixture is molded and sintered to produce a sintered body having density of the order of 5.0 - 7.2 g/cm³ usually. The utilization of such powder metallurgy makes it possible to produce an extremely complicated configuration of mechanical component with great accuracy in size. In a case where a mechanical component is to be produced with greater accuracy in size, it happens that a machine work, such as cutting, drilling or the like, is practiced on the sintered body.

Since products of the powder metallurgy or the sintered bodies are generally not excellent in machinability, a life-time of tools for use in cutting is shortened as compared with a case where wrought steel (e.g. materials obtained by means of rolling ingots produced through continuous casting) are subjected to cutting. This involves such a problem that the cost for the above-mentioned machine work is increased. The cause that machinability of the sintered body is low resides in pores included in the sintered body. The pores cause the cutting to be intermittently, or cause a coefficient of thermal conductivity of the sintered body to go down thereby increasing a temperature of the cutting section.

In view of the foregoing, hitherto, in many case, sulphur (S) or manganous sulfide (MnS) is mixed with iron powder in order to improve machinability of the sintered body. The reasons why it is to do so is that those sulphur (S) and manganous sulfide (MnS) make it easy to perform cutting out of chips, or form a thin film of sulphur (S) or manganous sulfide (MnS) on a tool cutting face, so that the thus formed thin film exhibits a lubrication action.

For example, Japanese Patent Publication (Kokoku) Hei.3-25481 proposes iron powders for powder metallurgy which are produced by means of atomizing with water or gas a molten steel in which 0.03-0.07 weight % of S is added to pure iron containing 0.1-0.5 weight % of Mn, Si and C. However, machinability of the sintered body produced by the use of such iron powders is simply improved by about twice or less as compared with that produced by the use of the conventional iron powders. Thus, the more improvement has been required in this respect.

Further, Japanese Patent Application Laid Open Gazette (Kokai) Sho.61-253301 proposes alloy steel powders comprising: at least one type of components of not more than 0.10 wt% of C, not more than 2.0 wt% of Mn, not more than 0.30 wt% of O, 0.10-5.0 wt% of Cr, 0.10-5.0 wt% of Ni, not more than 2.0 wt% of Si, 0.10-10.0 wt% of Cu, 0.01-3.0 wt% of Mo, 0.01-3.0 wt% of W, 0.01-2.0 wt% of V, 0.005-0.50 wt% of Ti, 0.005-0.50 wt% of Zr, 0.005-0.50 wt% of Nb,0.03-1.0 wt% of P and 0.0005-1.0 wt% of B; if necessary, not more than 1.0 wt% of S; and the remains which are substantially Fe.

However, the alloy steel powders are produced in such a manner that iron powders, which are formed through a rough reduction of iron oxide such as iron ore, mill oxide and the like, and mother alloy powders, which are formed through a water-atomizing of molten steels pre-alloyed with a lot of metallic elements, are mixed with one another and the thus mixed powders are subjected to a finish reduction process. Consequently, such alloy steel powders are produced in a very complicated scheme, and in addition contain a lot of alloy elements in large quantities. Thus, such alloy steel powders are expensive. Incidentally, the above-mentioned mother alloy powders formed through the water-atomizing comprises: at least one type of components of not more than 0.50 wt% of C, not more than 5.0 wt% of Mn, not more than 1.5 wt% of O, 0.10-20.0 wt% of Cr, 0.15-20.0 wt% of Ni, not more than 5.0 wt% of Si, 0.15-20.0 wt% of Cu, 0.015-15.0 wt% of Mo, 0.015-15.0 wt% of W, 0.015-5.0 wt% of V, 0.01-2.0 wt% of Ti, 0.01-2.0 wt% of Zr, 0.01-2.0 wt% of Nb, 0.04-2.0 wt% of P and 0.0010-2.0 wt% of B; if necessary, not more than 4 wt% of S; and the remains which are substantially Fe.

Then, as disclosed in Japanese Patent Application Laid Open Gazette (Kokai) Hei.7-233401 and Japanese Patent Application Laid Open Gazette (Kokai) Hei.7-233402, Applicant proposed water-atomized steel powders containing S,Cr and Mn in which machinability and abrasion resistance of sintered bodies are somewhat improved as compared with the prior art. At that time, the Applicant clarified that there was a remarkable improvement in the machinability of the sintered bodies, in view of the fact that when such steel powders were sintered, graphite remains in pores of the sintered bodies, and in addition MnS deposits on iron particles. Incidentally, it is considered that the reason why graphite remains in the pores is that in the sintering procedure Cr and S suppress the diffusion of graphite into iron powder particles.

However, even in case of such steel powders, containing H₂ in atmosphere gas at the time of sintering causes such a problem that machinability and abrasion resistance of sintered bodies are degraded. Thus, further improvement was desired.

In view of the foregoing, Applicants proposed in Japanese Patent Application SN. Hei.7-15368 a technology in which an amount of residual graphite is increased by means of sintering iron powders containing 0.001-0.03 wt% of B, 0.02-0.07 wt% of Cr, less than 0.1 wt% of Mn, and 0.03-0.15 wt% of one or more types of S, Se and Te on a total basis.

However, according to the technology mentioned above, an amount of residual graphite was about 0.42 wt% in the maximum, and composition of iron powders including above 0.03 wt% of B and above 0.1 wt% of Mn involved no improvement of machinability.

Then, there is desired iron powders capable of producing sintered steels containing a large amount of graphite in sintered bodies.

### Disclosure of the Invention

In view of the foregoing, it is an object of the present invention to provide iron powders for powder metallurgy, which are capable of producing sintered bodies exhibiting more excellent machinability and abrasion resistance as compared with the prior art, a method of producing such iron powders, and mixed powders in which other powders are added to the iron powders.

Taking into consideration the matters described in Japanese Patent Application Laid Open Gazette (Kokai) Hei.7-233401 and Japanese Patent Application Laid Open Gazette (Kokai) Hei.7-233402, the inventors of the present application studied as to how machinability and abrasion resistance of the sintered bodies are improved. In other words, the inventors made efforts diligently to discover alloy elements capable of more increasing an amount of residual graphite as compared with the sintered bodies. As a result, the inventors obtained such a new knowledge that sintering molten steels containing boron (B) and not larger than 100ppm of oxygen using iron powders subjected to a water-atomizing procedure causes an amount of residual graphite to be dramatically increased. Further, an important feature of the present invention resides in the point that segregation of boron (B) not less than a predetermined amount on surfaces of the iron powders is induced. The present invention is to embody the above-mentioned knowledge. That is, according to the present invention, there is provided an iron powder for powder metallurgy characterized in that the iron powder comprises 0.03 - 0.3 wt% of B, not more than 0.07 wt% of Cr, less than 0.3 wt% of Mn, and a balance being Fe and inevitable impurities, and an intensity ratio of Fe and B as to an emission spectrum obtained through a measurement on a surface of the iron powder according to Auger electron spectroscopy is not less than 0.05.

Further, there is provided an iron powder for powder metallurgy characterized in that in addition to the above-mentioned compositions, said iron powder further comprises 0.001 - less than 0.20 wt% in total of one or more of S, Se and Te, or comprises 0.05 - 3.5 wt% of Mo.

Furthermore, there is provided an iron base mixed powder for powder metallurgy characterized in that 0.05 - 0.7 wt% of MoO₃ powder and/or 0.05 - 0.7 wt% of WO₃ powder are mixed with the iron powder mentioned above.

Still furthermore, there is provided a method of producing iron powders for powder metallurgy, characterized in that a molten steel, which comprises 0.03 - 0.3 wt% of B, not more than 0.07 wt% of Cr, less than 0.3 wt% of Mn, not more than 100ppm of oxygen, and a balance being Fe and inevitable impurities, is used, said molten steel is water-atomized into powders, and the powders are sequentially subjected to dehydration dry and reduction treatments.

In addition, there is provided a method of producing iron powders for powder metallurgy characterized in that in addition to the above-mentioned compositions, said molten steel further comprises 0.001 - less than 0.20 wt% in total of one or more of S, Se and Te, or comprises 0.05 - 3.5 wt% of Mo.

According to the present invention, there are provided iron powders for powder metallurgy capable of easily producing sintered bodies having excellent machinability and abrasion resistance as compared with prior art.

### Brief Description of the Drawings

Fig. 1 is a view showing, by way of example, emission spectrum obtained through measurement of surfaces of iron powders related to the present invention by Auger electron spectroscopy.

Fig. 2 is a graph showing examples of concentration distributions of elements of interest at positions in depth direction from surfaces of iron powders measured by Auger electron spectroscopy. Incidentally, sputtering time of the abscissa axis is associated with a distance in depth direction from surfaces of iron powders.

### Best Mode for Carrying Out the Invention

According to the present invention, there is provided such a process that the content of Cr and Mn in iron powders is suppressed to be little, and to the contrary, the content of boron (B) is actively increased, so that segregation of boron (B) on surfaces of the iron powders may be induced. As a result, an amount of residual graphite contained in sintered bodies produced with the thus obtained iron powders is increased as compared with the conventional sintered bodies, thereby improving machinability. And in addition, there is also improved abrasion resistance of the sintered bodies by the self lubrication action of the residual graphite. It is considered that an amount of residual graphite is increased, because a water-atomizing of a molten steel containing boron (B) makes part of B to be easily oxidized through water and be deposited on surfaces of iron powders in the form of boron oxides, and the thus formed boron oxides serve to suppress the diffusion of C into the iron powders during the sintering.

A first important feature of the present invention resides in the point that a molten steel, in which the content of oxygen is below 100ppm, is atomized. A second important feature of the present invention resides in the point that a degree of segregation of boron (B) on surface of iron powders is defined as claimed. Those two features of the invention make it possible to increase an amount of residual graphite with a high B composition and a low B composition as compared with that of Japanese Patent Application SN. Hei.7-15368, thereby implementing improvements of machinability and abrasion resistance. Especially, it is noted that when an amount of graphite contained in sintered bodies is above 1 wt%, abrasion resistance is dramatically improved.

Further, according to the present invention, the combination use of S, Se and Te with the above-mentioned boron (B) promotes the effects mentioned above. Furthermore, according to the present invention, there is proposed iron powders containing Mo. Incidentally, it is more effective in improvement of machinability of sintered bodies that MoO₃ powders are mixed with the above-mentioned iron powders according to the present invention, rather than that Mo is added at stage of the molten steel through a process in which Mo is pre-alloyed. Since WO₃ powders also exhibit the similar effect to MoO₃ powders, such WO₃ powders are involved in the present invention.

Consequently, when iron powders for powder metallurgy or iron base mixed powders according to the present invention are mixed with copper powders or graphite powders in accordance with the usual way to form pressure molding bodies, and the thus formed pressure molding bodies are sintered, it is possible to easily produce sintered bodies containing a large quantity of residual graphite, the sintered bodies being excellent in machinability and abrasion resistance. Hereinafter, the reasons why the contents of elements of interest are restricted will be described.

### B: 0.03 - 0.3 wt%

Part of B added to molten steels is deposited on surfaces of iron powders in the form of an oxide, when the molten steel is atomized. And when the green compact of the iron powders is sintered, the oxide serves to suppress a diffusion of carbon into iron particles, so that an amount of residual graphite in the sintered body is increased. As a result, it is possible to improve machinability and abrasion of the sintered body. Further, boron oxides are very stable in chemistry and does not react with H₂. Thus, even if the sintering is performed in hydrogen atmosphere, this involves no deterioration of machinability of the sintered body as in the case of the steel powders disclosed in Japanese Patent Application Laid Open Gazette (Kokai) Hei.7-233401. It is noted that an adoption of a scheme such that Fe-B alloy powders are simply mixed with iron powders containing no B did not bring about an increase of an amount of residual graphite in the sintered body, and thus did not involve an improvement of machinability and the like.

Containing B not less than 0.03 wt% causes an amount of residual graphite to be extremely increased, and as a result, it is possible to improve machinability and abrasion of the sintered body. Thus, according to the present invention, 0.03 wt% of B is determined as the lower limit. On the other hand, when the content of B exceeds 0.3 wt%, part of B is solid-soluted on iron powder particles, so that hardness of the sintered body is increased thereby deteriorating the machinability. Thus, according to the present invention, 0.3 wt% of B is determined as the upper limit.

B on surfaces of iron powders: above 0.05 in intensity ratio of B to Fe as to emission spectrum derived through a measurement by Auger electron spectroscopy

As mentioned above, segregation of B on surfaces of iron powders causes an amount of residual graphite to be increased. Such B segregated on the surfaces of the iron powders can be confirmed through a measurement by Auger electron spectroscopy. Fig. 1 shows by way of example emission spectrum derived through the measurement.

The inventor evaluated the intensity ratio of B to Fe from the spectrum as shown in Fig. 1. Specifically, the intensity ratio of B to Fe implies the ratio of a peak-to-peak value of B corresponding to electronic energy 179eV (abscissa axis) to a peak-to-peak value of Fe corresponding to electronic energy 703eV. According to the study of the inventor, while an amount of residual graphite in the sintered body is increased in case of not less than 0.05 in the intensity ratio of B to Fe, it is not so in case of less than 0.05. Thus, according to the present invention, it is the condition for iron powders that the intensity ratio of B to Fe is not less than 0.05.

As the confirmation, there is shown in Fig. 2 examples of concentration distributions of elements of interest at positions in depth direction from surfaces of iron powders measured by Auger electron spectroscopy. Incidentally, sputtering time of the abscissa axis is associated with a distance in depth direction from surfaces of iron powders. In Fig. 2, concentration of B on surfaces of iron powders is 17 % by atomic weight %. It is considered that B exists in the form of B₂O₃ since oxygen is also concentrated together with B on the surfaces thereof.

Incidentally, in a qualitative analysis of iron powders according to Auger electron spectroscopy adopted in the present invention, accelerating voltage of the primary electron beam was 10kV, and beam current was 1.1µ A. And reading of the measured data was performed by 1.00eV/step and 50m sec/step; integration was performed eleven times; and five points differentiation was practiced to generate differential spectrum.

### Cr: below 0.07 wt%

Cr is easy to form oxides and covers surfaces of iron powders, thereby hindering surface segregation of B. Thus, it is necessary to limit the content of Cr as little as possible. Further, Cr forms carbide, so that hardness of sintered bodies is increased, thereby degrading machinability. For these reasons, according to the present invention, it is determined that Cr is not more than 0.07 wt%. Taking into account machinability and abrasion of the sintered body, and a manufacturing cost as well, it is preferable that Cr is 0.02 - 0.06 wt%.

### Mn: less than 0.3 wt%

Mn is an element which serves to reduce residual graphite. Further, when Mn in iron powder particles reacts with S, Se and Te, compounds are formed. Such compounds serve to reduce S, Se and Te which are effective to increase residual graphite in sintered bodies. Furthermore, Mn forms oxides and covers surfaces of iron powders, thereby hindering segregation of B on the surface of the iron powder. For these reasons, containing not less than 0.3 wt% of Mn causes reduction of residual graphite in sintered bodies. This involves deterioration of machinability. Taking into account the refining cost required for reduction of an amount of Mn in the regulation step of the molten steel component, and machinability of the sintered body, it is preferable that Mn is 0.07 - 0.15 wt%.

### Total of one or more of S, Se and Te : 0.001 - less than 0.20 wt%

S, Se and Te are contained in order to increase an amount of residual graphite in sintered bodies. The total amount of S, Se and Te is limited to 0.001 - less than 0.20 wt%. When the total amount of S, Se and Te exceeds 0.20 wt%, "soot" occurs. This makes mechanical parts as products easy to get rusty. For this reason, 0.20 wt% is determined as the upper limit. On the other hand, less than 0.001 wt% involves no effect of increasing an amount of residual graphite. Thus, the range of 0.001 - less than 0.20 wt% is determined.

### Mo: 0.05 - 3.5 wt%

Mo is contained in order to increase strength of iron powders. However, less than 0.05 wt% of Mo involves no improvement of strength of iron powders. On the other hand, exceeding 3.5 wt% of Mo involves rapid deterioration in machinability of sintered bodies. For these reasons, the above-noted range is determined. Incidentally, taking into account strength and machinability, the preferable range is 0.4 - 0.7 wt%.

### Total amount of MoO₃ powders and/or WO₃ powders: 0.05 - 0.7 wt%

MoO₃ powders and/or WO₃ powders are mixed with the above-mentioned iron powders according to the present invention so as to be utilized to form new mixed powders for powder metallurgy. Objects of the mixture are to improve machinability of sintered bodies and increase strength thereof by solid-solution hardening. Less than 0.05 wt% of total amount of MoO₃ powders and/or WO₃ powders involves no effects as mentioned above. On the other hand, exceeding 0.7 wt% of total amount of MoO₃ powders and/or WO₃ powders causes bainite to produce in iron particles, so that strength of the sintered body is deteriorated. For this reason, the total amount of MoO₃ powders and/or WO₃ powders is limited to the range of 0.05 - 0.7 wt%.

When above MoO₃ and/or WO₃ powders, graphite powders and copper powders are mixed with iron powders. The mixing for this invention is preferable to be done by the well known segregation preventing treatments (cf.Japanese Patent Application Laid Open Gazette (Kokai) Hei.1-165701 and Japanese Patent Application Laid Open Gazette (Kokai) Hei.2-47201). The reason why it is to do so is that MoO₃ powders and/or WO₃ powders are mixed homogeneously with iron powders, so that solid solution of Mo and/or W onto the iron powders within sintered bodies is performed homogeneously as compared with a simple mixing scheme. As a result, after sintered, the ferrite phase within sintered bodies becomes fine. This causes strength of the sintered body to increase by about 15 % as compared with a case where it is produced in accordance with a simple mixing scheme.

### Oxygen in molten steel: Below 100ppm

Iron powders according to the present invention are formed by way of water-atomizing molten steels controlled in the above-mentioned composition range. At that time, an amount of Oxygen (O) in the molten steel is determined to be below 100ppm, and preferably to be below 70ppm. Exceeding 100ppm of an amount of Oxygen (O) in the molten steel brings about a slagging by change of boron (B) into B₂O₃. This causes an amount of boron (B) effective for iron powders to decrease. For this reason, it is important that an amount of Oxygen (O) in the molten steel is limited as little as possible; Boron is molten in the molten steel and thereafter atomized; and the thus processed B is segregated on surfaces of iron powders in the form of B and B₂O₃ through oxidizing of B with water.

The iron powders formed by the water-atomizing process are subjected to dry, dehydration and reduction treatments as usual, and then crushed and classified to form iron powders.

### Embodiment 1

Applicant produced nine types of iron powders each type comprising B: 0.02 - 0.10 wt%, Cr: 0.02 - 0.04 wt%, Mn: 0.06 - 0.07 wt%, and the remainder of Fe and unavoidable impurity. In detail, the above-mentioned nine types of iron powders comprise five types of iron powders according to the present invention, and four types of iron powders (hereinafter, referred to as comparative examples) for comparison with the embodiment. A method of producing those types of iron powders is as follows.

First, a molten steel of temperature 1630°C given with a predetermined composition was water-atomized to form powders. The thus obtained powders were dried at 140°C for 60 minutes under a nitrogen atmosphere, and then subjected to a reduction treatment at 930°C for 20 minutes under a pure hydrogen atmosphere. And after cooling, the powders taken out from a reducing furnace were crushed and classified to form items Nos. 1-6 shown in Table 1.

In accordance with the same method of producing, there were produced iron powders further containing S: 0.02 - 0.10 wt% in addition to the composition of the above-mentioned iron powders. These are items Nos. 7-10 shown in Table 1. Incidentally, the molten steel before atomizing is one in which iron containing carbon is added and the content of oxygen is controlled to a range of 40 -200 ppm.

As to surfaces of items of Nos. 1-9 thus produced, emission spectrums were measured in accordance with Auger electron spectroscopy, and an intensity ratio of peak-to-peak (179eV) of B and peak-to-peak (703eV) of Fe was calculated. A measurement method and measurement conditions are the same as the above-mentioned ones.

Next, 1.2 wt% of graphite powders, 2.0 wt% of copper powders and 1 wt% of zinc stearate were mixed with those iron powders. Thereafter columnar green compacts were formed under pressure to 6.85 g/cm³ of density. These green compacts were sintered at 1130 °C for 20 minutes under a nitrogen atmosphere.

An amount of residual graphite in the obtained sintered body was evaluated as follows. The content of residue which is obtained by dissolving the sintered bodies in nitric acid and filtrating with glass filter was measured by infrared-absorbing method. With respect to machinability of the sintered body, it was estimated in such a manner that those iron powders were used to additionally produce a columnar sintered body of an external diameter of 60mm ⌀ and a height of 10mm, and the thus obtained sintered body is adopted as a sample. Concretely, first, a drill made of high-speed steel having 2 mm ⌀ in diameter was rotated under the conditions of 10000 rpm and 0.012 mm/rev to form a lot of apertures on the sample. And there was evaluated an average number of pieces (average value on three drills) in aperture until the drill become impossible to work. It is considered that the sample of the sintered bodies is more excellent in machinability with larger number of average value (it implies that the life-time of the tool is long).

Properties of the above-explained iron powders and sintered bodies are shown in Table 1.

As apparent from Table 1, according to the sintered body produced with the iron powders for powder metallurgy according to the present invention, oxygen in the molten steel is given below 100 ppm. Consequently, intensity ratios of B to Fe as to spectrum obtained through a measurement on surfaces of iron powders by Auger electron spectroscopy are not less than 0.05. Further, an amount of residual graphite of the sintered bodies is larger as compared with the comparative examples, thereby improving well machinability of the sintered bodies.

### Embodiment 2

Applicant further produced many types of atomized iron powders each comprising compositions shown in Table 2. In detail, the above-mentioned types of iron powders comprise six types (Nos. 11, 12, 16, 18, 23 and 24) of iron powders according to the present invention, four types of iron base mixed powders (Nos. 13, 14, 15 and 17) and four types of comparative examples (Nos. 19 - 22). Table 2 shows also an amount of oxygen in molten steels before water-atomized.

Those iron powders and iron base mixed powders were processed in similar treatment to that of embodiment 1, and thereafter a spectrum intensity ratio of peak-to-peak (179eV) of B to peak-to-peak (703eV) of Fe on surfaces of the iron powders was measured in accordance with Auger electron spectroscopy. Under the same conditions as embodiment 1, sintering of green compacts was performed, an amount of residual graphite of the thus obtained sintered body was measured and machinability was estimated.

It will be understood from Table 2 that the sintered bodies produced with the atomized iron powders and the iron base powders according to the present invention include a large amount of residual graphite, elongate life-times of tools, and are excellent in machinability.

### Embodiment 3

Applicant produced several types of atomized iron powders each comprising compositions shown in Table 3. In detail, the above-mentioned types of iron powders comprise four types (Nos. 25 - 28) of iron powders according to the present invention and four types of comparative examples (Nos. 29 - 31). 2 wt% of graphite powders and 15 wt% of copper powders were mixed with those iron powders, and as lubricant 1 wt% of zinc stearate was added and thereafter green compacts were formed under pressure to 6.85 g/cm³ of density. Next, these green compacts were sintered at 1130 °C for 20 minutes under an RX (endothermic gas) atmosphere.

Table 3 shows also an amount of residual graphite in the obtained sintered bodies and a spectrum intensity ratio of B to Fe according to Auger electron spectroscopy mentioned above. The applicant produced a cylindrical test sample of inside diameter 10mm⌀ x outside diameter 20mm⌀ x height 8mm, and inserted a shaft made of S45C of diameter 10mm⌀ into the cylinder with a clearance 20µm as to the inside wall. And an abrasion resistance test was performed in such a way that the shaft was rotated at 100 m/min by circumferential speed under dry conditions and load was increased gradually from the light load. In other words, the load at the time when sticking has occurred between the shaft and the inside wall of the cylinder is selected as the abrasion resistance index.

Items Nos. 25 - 28 of iron powders according to the present invention have an abrasion resistance not less than 4 kgf/cm² by load. As apparent from the above, when an amount of graphite in the sintered bodies is not less than 1 wt%, the abrasion resistance is extremely improved. On the other hand, item No. 29 of iron powders noted as the comparative example is few in segregation of B; item No. 30 of iron powders does not contain B; and item No. 31 of iron powders contain too much B. Thus, abrasion resistances of the sintered bodies produced with the use of those materials are inferior as compared with the iron powders according to the present invention.

**Table 3**

| No. | Chemical Components (wt %) | | | | B/Fe Intensity Ratio | Amount of Residual Graphite wt % | Abrasion Resistance kgf/cm² | Remarks |
|---|---|---|---|---|---|---|---|---|
| | B | Cr | Mn | S | | | | |
| 25 | 0.050 | 0.06 | 0.06 | 0.002* | 0.10 | 1.0 | 4.0 | Inventive Example |
| 26 | 0.100 | 0.03 | 0.07 | 0.08 | 0.06 | 1.7 | 7.0 | Inventive Example |
| 27 | 0.150 | 0.02 | 0.04 | 0.03 | 0.10 | 1.8 | 8.0 | Inventive Example |
| 28 | 0.180 | 0.02 | 0.05 | 0.10 | 0.09 | 1.8 | 8.3 | Inventive Example |
| 29 | 0.050 | 0.06 | 0.07 | 0.002* | 0.02 | 0.5 | 2.0 | Comparative Example |
| 30 | - | 0.06 | 0.07 | 0.03 | N.D | 0.02 | 0.2 | Comparative Example |
| 31 | 0.500 | 0.06 | 0.06 | 0.002* | 0.10 | 0.8 | 0.7 | Comparative Example |

| | | | | | | | | |
|---|---|---|---|---|---|---|---|---|
| * Inevitable impurities | | | | | | | | |

### Industrial Applicability

Iron powders for powder metallurgy and iron base mixed powders according to the present invention are more excellent in machinability and abrasion resistance of sintered bodies as compared with the conventional iron powders and mixed powders, when those powders are sintered in the form of green compacts. Consequently, when those powders are used to produce mechanical parts in accordance with a method of powder metallurgy of concern, it is possible to increase a dimensional accuracy of the mechanical parts and elongate the life-time thereof. Thus, the present invention is very useful in an industry.

## Claims

1. An iron powder for powder metallurgy characterized in that the iron powder comprises 0.03 - 0.3 wt% of B, not more than 0.07 wt% of Cr, less than 0.3 wt% of Mn, and a balance being Fe and inevitable impurities, and a ratio of a peak-to-peak value of B to a peak-to-peak value of Fe as to an emission spectrum obtained through a measurement on a surface of the iron powder according to Auger electron spectroscopy is not less than 0.05.

2. An iron powder for powder metallurgy according to claim 1, characterized in that said iron powder further comprises 0.001 - less than 0.2 wt% in total of one or more of S, Se and Te.

3. An iron powder for powder metallurgy according to claims 1 or 2, characterized in that said iron powder further comprises 0.05 - 3.5 wt% of Mo.

4. An iron base mixed powder for powder metallurgy characterized in that 0.05 - 0.7 wt% of MoO₃ powder and/or 0.05 - 0.7 wt% of WO₃ powder are mixed with the iron powder defined in claims 1 or 2.

5. A method of producing iron powders for powder metallurgy, characterized in that a molten steel, which comprises 0.03 - 0.3 wt% of B, not more than 0.07 wt% of Cr, less than 0.3 wt% of Mn, not more than 100ppm of oxygen, and a balance being Fe and inevitable impurities, is used, said molten steel is water-atomized into powders, and the powders are sequentially subjected to dehydration dry and reduction treatments.

6. A method of producing iron powders for powder metallurgy according to claim 5, characterized in that said molten steel further comprises 0.001 - less than 0.2 wt% in total of one or more of S, Se and Te.

7. A method of producing iron powders for powder metallurgy according to claims 5 or 6, characterized in that said molten steel further comprises 0.05 - 3.5 wt% of Mo.
